

## United States Patent [19]

Land et al.

[11] 3,833,368

[45] Sept. 3, 1974

[54] PHOTOGRAPHIC PRODUCTS  
INCORPORATING ANTI-REFLECTION  
COATINGS[75] Inventors: **Edwin H. Land**, Cambridge; **Stanley M. Bloom**, Waban, both of Mass.[73] Assignee: **Polaroid Corporation**, Cambridge, Mass.[22] Filed: **Dec. 4, 1972**[21] Appl. No.: **311,831**

[52] U.S. Cl. .... 96/3, 96/29 D, 96/29 R, 96/67, 96/76 R, 96/77, 96/84 R, 96/87 R, 96/119 R, 117/70 S, 117/72 R, 117/76 F

[51] Int. Cl. .... G03c 7/00, G03c 5/54, G03c 1/76, G03c 1/48, G03c 1/40, G03c 1/84, G03c 1/78, B41m 1/18

[58] Field of Search..... 117/705, 72 R, 76 P, 76 F; 96/3, 29 D, 29 R, 67, 76 R, 77, 87 R, 84 R

## [56] References Cited

## UNITED STATES PATENTS

|           |         |                      |          |
|-----------|---------|----------------------|----------|
| 2,536,764 | 1/1951  | Moulton .....        | 117/69   |
| 2,782,676 | 2/1957  | Osterberg.....       | 117/71 R |
| 3,526,530 | 9/1970  | Sams et al. ....     | 117/70 S |
| 3,617,354 | 11/1971 | Carnahan et al. .... | 117/76 P |

3,655,604 4/1972 Strolle..... 117/72 R  
3,754,924 8/1973 DeGeest et al. .... 96/67

Primary Examiner—David Klein

Assistant Examiner—Richard L. Schilling

Attorney, Agent, or Firm—Stanley H. Mervis

## [57] ABSTRACT

Photographic images, particularly multicolor images, viewed through a transparent support have an anti-reflection coating on the outer surface of said support. The anti-reflection coating comprises an eighth-wave layer of silica and an eighth-wave layer of a fluorinated polymer. The images may be formed by multicolor diffusion transfer processes using dye developers or other image dye-providing materials. In the preferred embodiments, the photographic image is an integral negative-positive reflection print. Where photoexposure is effected through a transparent support, e.g., the transparent support through which the final image is viewed, provision of an anti-reflection coating and effecting photoexposure therethrough will permit more effective recording of light passing through the camera lens. The transparent support preferably has an index of refraction of at least 1.6.

60 Claims, 5 Drawing Figures





SHEET 2 OF 4



FIG. 2

SHEET 3 OF 4



FIG. 3



FIG. 4

PATENTED SEP 3 1974

3,833,368

SHEET 4 OF 4



## PHOTOGRAPHIC PRODUCTS INCORPORATING ANTI-REFLECTION COATINGS

This invention is concerned with photography and, more particularly, with the formation of images in color or black-and-white by diffusion transfer processing.

A number of photographic processes have been proposed wherein the resulting photograph comprises the developed silver halide emulsion(s) retained as part of a permanent laminate, with the desired image being viewed through a transparent support. Of particular significance are those processes where the image is in color and is formed by a diffusion transfer process. If the image is to be viewed as a reflection print, the image-carrying layer is separated from the developed silver halide emulsion(s) in said laminate by a light-reflecting layer, preferably a layer containing titanium dioxide. Illustrative of patents describing such products and processes are U.S. Pat. No. 2,983,606 issued Mar. 9, 1961 to Howard G. Rogers, U.S. Pat. Nos. 3,415,644, 3,415,645 and 3,415,646 issued Dec. 10, 1968 to Edwin H. Land, U.S. Pat. Nos. 3,594,164 and 3,594,165 issued July 20, 1971 to Howard G. Rogers, and U.S. Pat. No. 3,647,347 issued Mar. 7, 1972 to Edwin H. Land.

Referring more specifically to the aforementioned U.S. Pat. No. 3,415,644, said patent discloses photographic products and processes employing dye developers wherein a photosensitive element and an image-receiving layer are maintained in fixed relationship prior to photoexposure and this fixed relationship is maintained after processing and image formation to provide a laminate including the processed silver halide emulsions and the image-receiving layer. Photoexposure is made through a transparent (support) element and application of a processing composition provides a layer of light-reflecting material to provide a white background for viewing the image and to mask the developed silver halide emulsions. The desired color transfer image is viewed through said transparent support against said white background.

While such processes provide very useful and good quality images, it has been found that the full potential quality of the image is not obtained because the transparent support through which the image is viewed in fact reflects "white" light to the viewer's eyes. Furthermore, this property of reflecting some of the light incident on the surface of the transparent support adversely affects the ability of the film to record a subject when photoexposure is effected through such a transparent support.

In accordance with the copending application of Edwin H. Land, Stanley M. Bloom and Howard G. Rogers, Ser. No. 276,979 filed Aug. 1, 1972 (now U.S. Pat. No. 3,793,022 issued Feb. 19, 1974), the above-noted problems are substantially, if not completely, eliminated by the provision of an anti-reflection layer through which the image is viewed and/or photoexposure is effected. The present invention is directed toward improvements in the products and processes disclosed and claimed in said Ser. No. 276,979, and, in its more specific embodiments, provides novel anti-reflection coatings.

It is, therefore, a primary object of this invention to provide novel photographic products and processes which provide color or black-and-white images as part

of a permanent laminate, said laminate exhibiting substantially less surface reflection of incident light.

It is a further object of this invention to provide diffusion transfer images, particularly multicolor transfer images, which are viewed through a transparent element the outer surface of which carries an improved anti-reflection coating.

Yet another object of this invention is to provide diffusion transfer films which are exposed through a transparent support, the outer surface of which carries an anti-reflection coating of improved scratch resistance.

Further objects of this invention include the provision of novel anti-reflection coatings and of transparent supports carrying said anti-reflection coatings, such supports being particularly useful for carrying photographically useful layers.

Other objects of this invention will in part be obvious and will in part appear hereinafter.

20 The invention accordingly comprises the product possessing the features, properties and relation of components and the process involving the several steps and the relation and order of one or more of such steps with respect to each of the others which are exemplified in 25 the following detailed disclosure, and the scope of the application of which will be indicated in the claims.

For a fuller understanding of the nature and objects of the invention, reference should be had to the following detailed description of the invention taken in conjunction with the accompanying drawings wherein:

FIGS. 1 and 2 are diagrammatic, enlarged cross-sectional views of two embodiments of film units embodying the present invention, illustrating the arrangement of layers during the three illustrated stages of a 35 monochrome diffusion transfer process, i.e., exposure, processing and final image;

FIG. 3 is a diagrammatic, enlarged cross-sectional view of another film unit embodying the present invention;

FIG. 4 is a diagrammatic, enlarged cross-sectional view of a transparent sheet, adapted for use as a support for an image-carrying element, including an anti-reflection coating in accordance with the present invention; and

FIG. 5 is a graph illustrating the anti-reflection properties of an anti-reflection coating of the type illustrated in FIG. 4.

As noted above, this invention is particularly concerned with color diffusion transfer processes wherein the layer containing the diffusion transfer image, i.e., the image-receiving layer, is not separated from the developed photosensitive layers after processing but both components are retained together as part of a permanent laminate. Film units particularly adapted to provide such diffusion transfer images have frequently been referred to as "integral negative-positive" film units. The resulting image may be referred to as an "integral negative-positive reflection print" and as so used this expression is intended to refer to a reflection print wherein the developed photosensitive layers have *not* been separated from the image layer, i.e., the layer containing the transfer dye image. A light-reflecting layer between the developed photosensitive layer(s) and the image layer provides a white background for the dye image and masks the developed photosensitive layer(s). These layers are part of a permanent laminate which usually includes dimensionally stable outer or

support layers, the transfer dye image being viewable through one of said supports. This invention is particularly concerned with improving the aesthetic qualities of such integral negative-positive reflection prints.

The present invention is applicable to a wide variety of diffusion transfer processes. The arrangement and order of the individual layers of the film used in such processes may vary in many ways as is known in the art, provided the final photograph is a laminate wherein the desired image is viewed through a transparent support, e.g., an integral negative-positive reflection print as described above. For convenience, however, the more specific descriptions of the invention hereinafter set forth will be by use of dye developer diffusion transfer color processes and of integral negative-positive film units of the type contemplated in the previously mentioned patents, particularly U.S. Pat. Nos. 3,415,644 and 3,594,164. It will be readily apparent from such descriptions that other image-forming reagents may be used, e.g., color couplers, coupling dyes or dyes (couplers) which release a dye or dye intermediate as a result of coupling or oxidation.

When such integral negative-positive reflection prints are viewed under ordinary lighting conditions, a small but significant amount of light is reflected from the external surface of the transparent support. The effect of this reflection of incident light is to limit the clarity with which the image may be seen except when the viewer's eyes are "just right," i.e., good viewing may be highly directional, in that the print may have to be "tilted" with respect to the viewer's line of vision to avoid obscuring image detail. This problem becomes more acute when several persons try to view the same image, as those not directly in front of the print will experience substantial glare, with the amount of glare increasing as the angle of view becomes more oblique. In addition, the color(s) of a color image may appear less saturated.

If photoexposure is effected through such a transparent support, reflection of light from the surface of the transparent support has been found to have several undesirable results. One result is a reduction in the exposure index or "speed" of the film, due to the fact that some of the light which has passed through the camera lens will be reflected before it can reach the photosensitive layer(s) and the thus reflected light will not participate in the recording of the photographed subject matter. Furthermore, such reflected light has a tendency to "bounce" within the camera, and may cause flare and reduced contrast and resolution in the final image. If photoexposure is effected through the transparent support in a camera which includes an image-reversing mirror in the optical path, light reflected from the surface may cause a "ghost" image of a particularly bright object within the scene to be superposed on another portion of the scene in the resulting photograph.

As noted earlier, the copending application of Land, et al., Ser. No. 276,979 teaches that such undesirable reflection from the transparent support may be substantially reduced, if not completely eliminated, by modifying the external surface of such transparent supports so as to provide a controlled change in the index of refraction to which incident light is subjected as it passes from air into the transparent support.

The present invention is directed towards perfecting the advantages provided by the teachings of Ser. No.

276,979 by providing improved anti-reflection coatings for use, e.g., on the external surface of the transparent support of a photographic element. In accordance with the present invention, an anti-reflection coating is provided which comprises an eighth-wave stratum of a fluorinated polymer over an eighth-wave stratum of silica, each said stratum having an optical thickness of one-eighth of substantially the same, predetermined wavelength of light. Especially good results are obtained when an eighth-wave coating of a low refractive index, fluorinated polymer is present over an eighth-wave coating of colloidal silica carried by a high refractive index, transparent synthetic polymeric sheet or support.

The principles of physics by which anti-reflection coatings function are well known and may be used to special advantage in the present invention. Thus, it is well known that application of a single layer transparent coating will reduce surface reflection from a transparent layer (support) if the refractive index of said coating is less than that of the transparent layer to which it is applied and the coating is of appropriate optical thickness. In the photographic products with which this invention is concerned, the anti-reflection coating will normally be in optical contact with air. Under these circumstances, and because the index of refraction of air is 1, the applicable principles of physics give the following rule: if the index of refraction of the coating material (anti-reflection layer) is exactly equal to the square root of the index of refraction of the substrate (transparent support), then all surface reflection of light will be eliminated for that wavelength at which the product of the refractive index times thickness is equal to one-quarter of that wavelength. At other wavelengths the destructive interference between light reflected from the top and bottom surfaces of the anti-reflection coating is not complete but a substantial reduction in overall reflectivity is obtained. By selecting the optical thickness of the anti-reflection coating to be one-quarter of a wavelength for approximately the midpoint of the visible light wavelength range (i.e., one-quarter of 5,500 Angstroms or about 1,400 Angstroms), the reduction in reflectivity is optimized. The term "optical thickness" as used herein refers to the product of the physical thickness of the coating times the refractive index of the coating material. Unless otherwise indicated, as used herein the expressions "eighth-wave" and "quarter-wave" refer to coatings having an optical thickness, respectively, of one-eighth and one-quarter of a predetermined wavelength of light, said wavelength being 5,500 Angstroms.

The anti-reflection coating should be optically clear and provide an essentially uniform layer. The anti-reflection coating may also be effective as an anti-abrasion coating, since it is preferably more scratch resistant than the support. While the above discussion of the applicable principles of physics has concerned itself with a single quarter-wave anti-reflection coating, it will be understood that the same principles are applicable to a anti-reflection coating comprising two eighth-wave strata where the indices of refraction of each eighth-wave stratum is within about 0.1 of the other.

Transparent supports with which the anti-reflection coatings of this invention may be used include polyesters, polystyrene, cellulose esters (such as cellulose acetate [triacetate] and cellulose acetate butyrate) polycarbonates, and similar art known polymeric film base

materials. Such film bases typically have a thickness of about 3 to 10 mils (0.003 to 0.010 inch). Particularly useful polyester film bases have a thickness of about 3 to 6 mils. Polyester and polystyrene films have higher refractive indices than cellulose acetate, and the resultant greater incidence of surface reflected light as compared with cellulose acetate would normally be considered to be a disadvantage of using such materials in integral negative positive reflection or other prints in which the image is viewed through a transparent base. (Indeed, the greater surface reflection resulting in greater glare, and the resultant need for more directional viewing, exhibited by polyester films as compared with cellulose acetate is well known from the commonly used protective transparent covers for notebook pages.) These higher indices of refraction are turned into an advantage by the present invention, for the high index of refraction makes it much more possible to provide anti-reflection coatings which practically eliminate all reflectivity, whereas reflectivity can only be reduced when using cellulose acetate.

Particularly useful transparent supports are films of polyethylene terephthalate, such as those commercially available under the trademarks "Mylar" (E. I. DuPont de Nemours & Co.) and "Estar" (Eastman Kodak Co.). Such polyester films have an index of refraction on the order of about 1.66. A number of materials suitable for anti-reflection coatings, e.g., fluorinated polymers, have indices of refraction of about 1.35 to 1.40 which is close to the 1.29 ideal index of refraction, i.e., the geometric mean of the indices of refraction of the polyethylene terephthalate and the surrounding air, or, because the index of refraction of air is 1, the square root of the 1.66 index of refraction of polyethylene terephthalate. Furthermore, the fact that the difference of about 0.3 in the indices of refraction between air and the anti-reflection coating is close to the approximate 0.3 difference in the indices of refraction of the anti-reflection coating and the polyethylene terephthalate support means that maximum benefit will be obtained from the anti-reflection coating; the amplitude of the light entering the anti-reflection coating will more closely match the amplitude of the light reflected back from the interface of the polyethylene phthalate and the anti-reflection coating, and more effectively cancel out the thus reflected light.

Reference is now made to the accompanying drawings wherein a plurality of embodiments of this invention are illustrated and wherein like numbers, appearing in the various figures, refer to like components. For ease of understanding, these embodiments illustrate the formation of a monochrome image using a single dye developer. The illustrated embodiments include appropriate means of opacification to permit the processing of the film unit outside of a dark chamber, i.e., the film unit is intended to be removed from the camera prior to image completion and while the film is still photosensitive. Opacifying systems are described in the previously noted patents and per se form no part of the present invention which is equally applicable to film units intended to be processed within a dark chamber.

In the discussion of FIGS. 1, 2 and 3, reference to the anti-reflection coating 26 is to be understood as referring to the anti-reflection coating provided by strata 26a and 26b of FIG. 4.

A particularly useful opacifying system for film units of the type shown in FIGS. 1 and 3 utilizes a color dischargeable reagent, preferably a pH-sensitive optical filter agent or dye, sometimes referred to as an indicator dye, as is described in detail in the aforementioned U.S. Pat. No. 3,647,437. In film units of the type shown in FIG. 2, photoexposure is effected from the side opposite the side from which the image is viewed. An opaque layer to protect the exposed silver halide from further exposure may be provided by including a light-absorbing opacifying agent, e.g., carbon black, in the processing composition which is distributed between the photosensitive layer(s) and a transparent support or spreader sheet. In such film units, it may be desirable to include a preformed opaque layer, e.g., a dispersion of carbon black in a polymer permeable to the processing composition, between a preformed light-reflecting layer and the silver halide emulsion(s). Such opacifying systems are shown and described in the aforementioned U.S. Pat. Nos. 3,594,164 and 3,594,165.

Referring to FIG. 1, Stages A, B and C show in diagrammatic cross-section, respectively, imaging, processing, and the finished print in one embodiment of this invention. In Stage A, there is shown a photosensitive element 30 in superposed relationship with an image-receiving element 32, with a rupturable container 16 (holding an opaque processing composition 17) so positioned as to discharge its contents between said elements upon suitable application of pressure, as by passing through a pair of pressure applying rolls or other pressure means (not shown). Photosensitive element 30 comprises an opaque support 10 carrying a layer 12 of a dye developer over which has been coated a silver halide emulsion layer 14. The image-receiving element 32 comprises a transparent support 24 carrying, in turn, a polymeric acid layer 22, a spacer layer 20 and an image-receiving layer 18. An anti-reflection coating 26 is present on the outer surface of the transparent support 24. Photoexposure of the silver halide emulsion layer is effected through the anti-reflection coating 26 and the transparent support 24 and the layers carried thereon, i.e., the polymeric acid layer 22, the spacer layer 20 and the image-receiving layer 18 which layers are also transparent, the film unit being so positioned within the camera that light admitted through the camera exposure or lens system is incident upon the outer surface of the anti-reflection coating 26. After exposure the film unit is advanced between suitable pressure-applying members, rupturing the container 16, thereby releasing and distributing a layer 17a of the opaque processing composition between the photosensitive element 30 and the image-receiving element 32. The opaque processing composition contains a film-forming polymer, a white pigment and has an initial pH at which one or more optical filter agents contained therein are colored; the optical filter agent (agents) is (are) selected to exhibit light absorption over at least a portion of the wavelength range of light actinic to the silver halide emulsion. As a result, ambient or environmental light within that wavelength range incident upon transparent support 24 and transmitted through said transparent support and the transparent layers carried thereon in the direction of the photoexposed silver halide emulsion 14a is absorbed thereby avoiding further exposure of the photoexposed and developing silver halide emulsion 14a. In exposed and developed areas, the dye developer is oxidized as a function of the

silver halide development and immobilized. Unoxidized dye developer associated with undeveloped and partially developed areas remains mobile and is transferred imagewise to the image-receiving layer 18 to provide the desired positive image therein. Permeation of the alkaline processing composition through the image-receiving layer 18 and the spacer layer 20 to the polymeric acid layer 22 is so controlled that the process pH is maintained at a high enough level to effect the requisite development and image transfer and to retain the optical filter agent (agents) in colored form, after which pH reduction effected as a result of alkali permeation into the polymeric acid layer 22 is effective to reduce the pH to a level which "discharges" the optical filter agent, i.e., changes it to a colorless form. Absorption of the water from the applied layer 17a of the processing composition results in a solidified film composed of the film-forming polymer and the white pigment dispersed therein, thus providing the reflecting layer 17b which also serves to laminate together the photosensitive element 30 and the image-receiving element 32 to provide the final laminate (Stage C). The positive transfer image in dye developer present in the image-receiving layer 18a is viewed through the transparent support 24 and the intermediate transparent layers against the reflecting layer 17b which provides an essentially white background for the dye image and also effectively masks from view the developed silver halide emulsion 14b and dye developer immobilized therein or remaining in the dye developer layer 12.

The optical filter agent is retained within the final film unit laminate and is preferably colorless in its final form, i.e., exhibiting no visible absorption to degrade the transfer image or the white background therefor provided by the reflecting layer 17b. The optical filter agent may be retained in the reflecting layer under these conditions, and it may contain a suitable "anchor" or "ballast" group to prevent its diffusion into adjacent layers. Alternatively, if the optical filter agent is initially diffusible, it may be selectively immobilized on the silver halide emulsion side of the reflecting layer 17b, e.g., by a mordant coated on the surface of the silver halide emulsion layer 14; in this embodiment the optical filter in its final state may be colorless or colored so long as any color exhibited by it is effectively masked by the reflecting layer 17b.

The reflecting layer provided in the embodiment of this invention shown in FIG. 1 is formed by solidification of a stratum of pigmented processing composition distributed after exposure. It is also within the scope of this invention to provide a preformed pigmented layer, e.g., coated over the image-receiving layer 18, and to effect photoexposure therethrough, in accordance with the teachings of U.S. Pat. No. 3,615,421 issued Oct. 26, 1971 to Edwin H. Land.

In the embodiment illustrated in FIG. 1, photoexposure is effected through the image-receiving element. While this is a particularly useful and preferred embodiment, it will be understood that the image-receiving element may be initially positioned out of the exposure path as illustrated in FIG. 3 and superposed upon the photosensitive element after photoexposure, in which event the processing and final image stages would be the same as in FIG. 1.

In the embodiment illustrated in FIG. 1, photoexposure and viewing of the final image both are effected through the transparent support 24. Accordingly, the

advantages of the anti-reflection coating 26 are obtained twice, i.e., first, by minimizing failure of the film unit to record light passed by the camera lens and second, by minimizing glare during viewing.

It will be noted in the embodiment illustrated in FIG. 1 that the image-viewing layer 18 is temporarily bonded to the silver halide emulsion layer 14 *prior to* exposure. The rupturable container or pod 16 is so positioned that upon its rupture the processing composition 17 will delaminate the film unit and distribute itself between the image-receiving layer 18 and the silver halide emulsion layer 14. The distributed layer of processing composition 17a upon solidification forms a layer 17b which bonds the elements together to form the desired permanent laminate. Procedures for forming such prelaminated film units, i.e., film units in which the several elements are temporarily laminated together prior to exposure, are described, for example, in U.S. Pat. No. 3,625,281 issued to Albert J. Barchelder and Frederick J. Binda and in U.S. Pat. No. 3,652,282 to Edwin H. Land, both issued Mar. 28, 1972. A particularly useful and preferred prelamination utilizes a water-soluble polyethylene glycol as described and claimed in the copending application of Edwin H. Land, Ser. No. 247,023 filed Apr. 24, 1972, now U.S. Pat. No. 3,793,623.

The use of such temporarily laminated film units maximizes the beneficial effects obtained in the photoexposure stage from having the exposure effected through the antireflection coating 26, since the prelamination eliminates any other layer-to-air interface which could also reflect light and thus reduce the amount of light recorded by the photosensitive layer(s).

It will be recognized that the transfer image formed following exposure and processing of film units of the type illustrated in FIG. 1 will be a geometrically reversed image of the subject. Accordingly, to provide geometrically nonreversed transfer images, exposure of such film units should be accomplished through an image reversing optical system, such as in a camera possessing an image reversing optical system utilizing mirror optics, e.g., as described in U.S. Pat. No. 3,447,437 issued June 3, 1969 to Douglas B. Tiffany. As noted above, when photoexposure is effected in such an image reversing optical system, photoexposure through an anti-reflection layer provides additional advantages in preventing the reflection of light which might cause the formation in the final image of a reflected or "ghost" image of one part of the photographed scene superposed upon another part of the scene.

If desired, the photosensitive element 30 may utilize a transparent support instead of the opaque support 10 shown in FIG. 1. In this alternative embodiment, the film unit should be processed in a dark chamber or an opaque layer, e.g., pressure-sensitive, should be superposed over said transparent support to avoid further exposure through the back of the film unit during processing outside of the camera.

FIG. 2 illustrates another film structure adapted to provide an integral negative-positive reflection print and wherein photoexposure and viewing are effected from opposite sides. In this embodiment, a photosensitive element 34 comprises a transparent support 24 carrying a layer 22 of a polymeric acid, a spacer 20, an image-receiving layer 18, a light-reflecting layer 60

(e.g., of titanium dioxide), an opaque layer 62 (e.g., of carbon black), a dye developer layer 12, and a silver halide emulsion layer 14. After photoexposure, a processing composition 17 is applied by rupturing a pod 16 and distributing the processing composition between a cover or spreader sheet 64 and silver halide emulsion layer 14. The cover sheet 64 may be transparent as illustrated in FIG. 2 and described in detail in the above noted U.S. Pat. No. 3,594,165, in which event photoexposure may be effected through it while it is held in place, e.g., by a binder tape around the edges of the film unit or by temporary lamination prior to photoexposure, as discussed above. In this embodiment, an anti-reflection coating 26 is provided on the outer or exposure surface of the transparent cover sheet 64. (Alternatively, cover sheet 64 may be opaque in which event it is positioned out of the exposure path prior to photoexposure, as described in detail in the above noted U.S. Pat. No. 3,594,164.) The opaque processing composition 17 contains suitable opacifying agents, e.g., carbon black, titanium dioxide, etc. The light-reflecting layer 60 preferably includes a white pigment, such as titanium dioxide, to provide a white background against which the transfer image may be viewed. The opaque layer 62, e.g., a layer of carbon black in gelatin, provides the requisite light protection while assuring an aesthetically pleasing white background for the final image.

Processing of film units of the types described above is initiated by distributing the processing composition between predetermined layers of the film unit. In exposed and developed areas, the dye developer will be immobilized as a function of development. In unexposed and undeveloped areas, the dye developer is unreacted and diffusible, and this provides an imagewise distribution of unoxidized dye developer, diffusible in the processing composition, as a function of the point-to-point degree of exposure of the silver halide layer. The desired transfer image is obtained by the diffusion transfer to the image-receiving layer of at least part of this imagewise distribution of unoxidized dye developer. In the illustrated embodiments, the pH of the photographic system is controlled and reduced by the neutralization of alkali after a predetermined interval, in accordance with the teachings of the above noted U.S. Pat. No. 3,615,644, to reduce the alkalinity to a pH at which the unoxidized dye developer is substantially insoluble and non-diffusible. As will be readily recognized, the details of such processes form no part of the present invention but are well known; the previously noted U.S. patents may be referred to for more specific discussion of such processes.

The film units illustrated in FIGS. 1, 2, and 3 have, for convenience, been shown as monochrome films. Multicolor images may be obtained by providing the requisite number of differentially exposable silver halide emulsions, and said silver halide emulsions are most commonly provided as individual layers coated in superposed relationship. Film units intended to provide multicolor images comprise two or more selectively sensitized silver halide layers each having associated therewith an appropriate image dye-providing material providing an image dye having spectral absorption characteristics substantially complementary to the light by which the associated silver halide is exposed. The most commonly employed negative components for forming multicolor images are of the "tripack" struc-

ture and contain blue-, green-, and red-sensitive silver halide layers each having associated therewith in the same or in a contiguous layer a yellow, a magenta and a cyan image dye-providing material respectively. Interlayers or spacer layers may, if desired, be provided between the respective silver halide layers and associated image dye-providing materials or between other layers. Integral multicolor photosensitive elements of this general type are disclosed in U.S. Pat. No. 3,345,163 issued Oct. 3, 1967 to Edwin H. Land and Howard G. Rogers as well as in the previously noted U.S. patents, e.g., in FIG. 9 of the aforementioned U.S. Pat. No. 2,983,606.

A number of modifications to the structures described in connection with the figures will readily suggest themselves to one skilled in the art. Thus, for example, the multicolor multilayer negative may be replaced by a screen-type negative as illustrated in U.S. Pat. No. 2,968,554 issued Jan. 17, 1961 to Edwin H. Land and in the aforementioned U.S. Pat. No. 2,983,606 particularly with respect to FIG. 3 thereof.

The image dye-providing materials which may be employed in such processes generally may be characterized as either (1) initially soluble or diffusible in the processing composition but are selectively rendered non-diffusible in an imagewise pattern as a function of development; or (2) initially insoluble or non-diffusible in the processing composition but which are selectively rendered diffusible or provide a diffusible product in an imagewise pattern as a function of development. These materials may be complete dyes or dye intermediates, e.g., color couplers. The requisite differential in mobility or solubility may, for example, be obtained by a chemical action such as a redox reaction or a coupling reaction.

As examples of initially soluble or diffusible materials and their application in color diffusion transfer, mention may be made of those disclosed, for example, in U.S. Pat. Nos. 2,774,668; 2,968,554; 2,983,606; 2,087,817; 3,185,567; 3,230,082; 3,345,163; and 3,443,943. As examples of initially non-diffusible materials and their use in color transfer systems, mention may be made of the materials and systems disclosed in U.S. Pat. Nos. 3,185,567; 3,443,939; 3,443,940; 3,227,550; and 3,227,552. Both types of image dye-providing substances and film units useful therewith also are discussed in the aforementioned U.S. Pat. No. 3,647,437 to which reference may be made.

It will be understood that dye transfer images which are neutral or black-and-white instead of monochrome or multicolor may be obtained by use of a single dye or a mixture of dyes of the appropriate colors in proper proportions, the transfer of which may be controlled by a single layer of silver halide, in accordance with known techniques. It is also to be understood that "direct positive" silver halide emulsions may also be used, depending upon the particular image dye-providing substances employed and whether a positive or negative color transfer image is desired.

It will also be understood that the present invention may be utilized with films wherein the final image is in silver, and photoexposure and/or viewing is effected through a transparent support which is provided with an anti-reflection coating in accordance with the teachings of this disclosure. Indeed, the transfer of silver may

be utilized to provide a silver image or to provide a dye image by silver dye bleach processing.

In the preferred embodiments, the layers comprising the individual film units are secured in fixed relationship prior to, during, and after photoexposure and processing to provide the desired integral negative-positive image. Film units of this type are well known in the art and are illustrated, for example, in the above cited U.S. Pat. Nos. 3,415,644; 3,467,437; and 3,594,165, as well as in other patents. In general, a binding member is provided extending around, for example, the edges of the composite structure and securing the elements thereof in fixed relationship. The binding member may comprise a pressuresensitive tape securing and/or maintaining the layers of the structure together at its respective edges. If the edge tapes are also opaque, edge leakage of actinic radiation incident on the film unit will be prevented. The edge tapes also will act to prevent leakage of the processing composition from the laminate during and after processing. The rupturable pod is so positioned as to discharge its contents between predetermined layers; e.g., between the image-receiving layer 18 and the silver halide emulsion layer 14 of FIG. 1; these layers may be temporarily bonded to each other with a bond strength less than that exhibited by the interface between the opposed surfaces of the remaining layers, as described above. The binding member may also serve to provide a white mask or border for the final image. The manufacture of such film units or packets is well described in the above-noted and other patents and need not be set forth in any detail here.

Rupturable container 16 may be of the type shown and described in any of U.S. Pat. Nos. 2,543,181; 2,634,886; 3,653,732; 2,723,051; 3,056,492; 3,056,491; 3,152,515; and the like. In general, such containers will comprise a rectangular blank of fluid- and air-impermeable sheet material folded longitudinally upon itself to form two walls which are sealed to one another along their longitudinal and end margins to form a cavity in which processing composition 17 is retained. The longitudinal marginal seal is made weaker than the end seals so as to become unsealed in response to the hydraulic pressure generated within the fluid contents 17 of the container by the application of compressive pressure to the walls of the container, e.g., by passing the film unit between opposed pressure applying rollers.

The rupturable container 16 is so positioned as to effect unidirectional discharge of the processing composition 17 between predetermined layers, e.g., the image-receiving layer 18 and the silver halide layer 14 next adjacent thereto, upon application of compressive force to the rupturable container 16. Thus, the rupturable container 16, as illustrated in FIG. 1, is fixedly positioned and extends transverse a leading edge of the prelaminated film unit with its longitudinal marginal seal directed toward the interface between the image-receiving layer 18 and the silver halide emulsion layer 14. The rupturable container 16 is fixedly secured to this laminate by a tape extending over a portion of one wall of the container, in combination with a separate retaining member or tape extending over a portion of the laminate's surface generally equal in area to about that covered by said tape.

A preferred opacification system to be contained in the processing composition 17 to effect processing outside of a camera is that described in the above-

mentioned U.S. Pat. No. 3,647,437, and comprises a dispersion of an inorganic light-reflecting pigment which also contains at least one light-absorbing agent, i.e., optical filter agent, at a pH above the pKa of the optical filter agent in a concentration effective when the processing composition is applied, to provide a layer exhibiting optical transmission density > than about 6.0 density units with respect to incident radiation actinic to the photosensitive silver halide and optical reflection density < than about 1.0 density units with respect to incident visible radiation.

In lieu of having the light-reflecting pigment in the processing composition, the light-reflecting pigment used to mask the photosensitive strata and to provide the background for viewing the color transfer image formed in the receiving layer may be present initially in whole or in part as a preformed layer in the film unit. As an example of such a preformed layer, mention may be made of that disclosed in U.S. Pat. No. 3,615,421 issued Oct. 26, 1971 and in U.S. Pat. No. 3,620,724 issued Nov. 16, 1971, both in the name of Edwin H. Land. The reflecting agent may be generated in situ as is disclosed in U.S. Pat. Nos. 3,647,434 and 3,647,435, both issued Mar. 7, 1972 to Edwin H. Land.

The dye developers (or other image dye-providing substances) are preferably selected for their ability to provide colors that are useful in carrying out subtractive color photography, that is, the previously mentioned cyan, magenta and yellow. They may be incorporated in the respective silver halide emulsion or, in the preferred embodiment, in a separate layer behind the respective silver halide emulsion. Thus a dye developer may, for example, be in a coating or layer behind the respective silver halide emulsion and such a layer of dye developer may be applied by use of a coating solution containing the respective dye developer distributed, in a concentration calculated to give the desired coverage of dye developer per unit area, in a film-forming natural, or synthetic, polymer, for example, gelatin, polyvinyl alcohol, and the like, adapted to be permeated by the processing composition.

Dye developers, as noted above, are compounds which contain the chromophoric system of a dye and also a silver halide developing function. By "a silver halide developing function" is meant a grouping adapted to develop exposed silver halide. A preferred silver halide development function is a hydroquinoyl group. Other suitable developing functions include ortho-dihydroxyphenyl and ortho-and para-amino substituted hydroxyphenyl groups. In general, the development function includes a benzenoid developing function, that is, an aromatic developing group which forms quinonoid or quinone substances when oxidized.

The image-receiving layer may comprise one of the materials known in the art, such as polyvinyl alcohol, gelatin, etc. It may contain agents adapted to mordant or otherwise fix the transferred images dye(s). Preferred materials comprise polyvinyl alcohol or gelatin containing a dye mordant such as poly-4-vinylpyridine, as disclosed in U.S. Pat. No. 3,148,061, issued Sept. 8, 1964 to Howard C. Haas.

In the various color diffusion transfer systems which have previously been described, and which employ an aqueous alkaline processing fluid, it is well known to employ an acid-reacting reagent in a layer of the film unit to lower the environmental pH following substantial dye transfer in order to increase the image stability

and/or to adjust the pH from the first pH at which the image dyes are diffusible to a second (lower) pH at which they are not. For example, the previously mentioned U.S. Pat. No. 3,415,644 discloses systems wherein the desired pH reduction may be effected by providing a polymeric acid layer adjacent the dyeable stratum. These polymeric acids may be polymers which contain acid groups, e.g., carboxylic acid and sulfonic acid groups, which are capable of forming salts with alkali metals or with organic bases; or potentially acid-yielding groups such as anhydrides or lactones. Preferably the acid polymer contains free carboxyl groups. Alternatively, or in addition, an acid-reacting reagent may be provided in a layer adjacent to the silver halide layer most distant from the image-receiving layer, as disclosed in U.S. Pat. No. 3,573,043 issued Mar. 30, 1971 to Edwin H. Land. Another system for providing an acid-reacting reagent is disclosed in U.S. Pat. No. 3,576,625 issued Apr. 27, 1971 to Edwin H. Land.

An inert interlayer or spacer layer may be and is preferably disposed between the polymeric acid layer and the dyeable stratum in order to control or "time" the pH reduction so that it is not premature and thus interfere with the development process. Suitable spacer or "timing" layers for this purpose are described with particularity in U.S. Pat. Nos. 3,362,819; 3,419,389; 3,421,893; 3,455,686; and 3,575,701.

While the acid layer and associated spacer layer are preferably contained in the positive component employed in systems wherein the dyeable stratum and photosensitive strata are contained on separate supports, e.g., between the support for the receiving element and the dyeable stratum; or associated with the dyeable stratum in those integral film units, e.g., on the side of the dyeable stratum opposed from the negative components, they may, if desired, be associated with the photosensitive strata, as is disclosed, for example, in U.S. Pat. Nos. 3,362,821 and 3,573,043. In film units such as those described in the aforementioned U.S. Pat. Nos. 3,594,164 and 3,594,165, they also may be contained on the spreader sheet employed to facilitate application of the processing fluid.

As is now well known and illustrated, for example, in the previously cited patents, the liquid processing composition referred to for effecting multicolor diffusion transfer processes comprises at least an aqueous solution of an alkaline material, for example sodium hydroxide, potassium hydroxide, and the like, and preferably possessing a pH in excess of 12, and most preferably includes a viscosity-increasing compound constituting a film-forming material of the type which, when the composition is spread and dried, forms a relatively firm and relatively stable film. The preferred film-forming materials comprise high molecular weight polymers such as polymeric, water-soluble ethers which are inert to an alkaline solution such as, for example, a hydroxyethyl cellulose or sodium carboxymethyl cellulose. Additionally, other film-forming materials or thickening agents whose ability to increase viscosity is substantially unaffected if left in solution for a long period of time are capable of utilization. The film-forming material is preferably contained in the processing composition in such suitable quantities as to impart to the composition a viscosity in excess of 100 cps. at a temperature of approximately 24° C. and preferably in the order of 100,000 cps. to 200,000 cps. at that temperature.

In particularly useful embodiments of this invention, the transparent support contains a small quantity of a pigment, e.g., carbon black, to prevent fog formation due to light-piping by internal reflection within the transparent support of actinic light incident upon an edge thereof; such elements are described and claimed in the copending application of Edwin H. Land Ser. No. 194,407 filed Nov. 1, 1971 (now abandoned and replaced by a continuation-in-part application, Ser. No. 419,808, filed Nov. 28, 1973). Similarly, fog from such lightpiping may be avoided by incorporating an alkali-dischargeable dye in a suitable layer, e.g., the image-receiving layer, in accordance with the disclosure of the copending application of Howard G. Rogers, Ser. No. 194,406 filed Nov. 1, 1971 (now abandoned and replaced by a continuation-in-part application, Ser. No. 408,052, filed Oct. 19, 1973). The transparent support advantageously may include an ultraviolet light absorber, as taught in the copending application of Ronald F. Cieciuch and Herbert N. Schlein, Ser. No. 214,600 filed Jan. 3, 1972 (now abandoned and replaced by a continuation-in-part application, Ser. No. 300,277, filed Oct. 24, 1972).

While it is generally desirable to provide the anti-reflection coating as part of the transparent support prior to applying the photographically used layers and subsequent assembly of the film unit, it is within the scope of this invention to apply the anti-reflection coating at any stage of the manufacture process that is best suited for the particular materials and components.

As discussed above, the anti-reflection coating or stratum should comprise a material having an index of refraction less than that of the transparent support. The optimum index of refraction to be exhibited by the anti-reflection coating may be readily calculated by the principles of physics previously discussed, but it is not essential that such optimum value be used in order to obtain very beneficial results. In the preferred embodiments of this invention, the transparent support is formed of a polymer having a high index of refraction, e.g., of about 1.6 or higher. The anti-reflection coating preferably has an index of refraction at least 0.20 less than, and more preferably at least 0.35 to 0.3 less than, the index of refraction of the transparent support. Since the preferred transparent supports will have an index of refraction of about 1.6 or higher, the preferred anti-reflection coatings will exhibit an index of refraction of about 1.3 to 1.45.

As stated above and as illustrated in FIG. 4, the novel anti-reflection coatings provided by this invention comprise an eighth-wave stratum of silica and an eighth-wave stratum of a fluorinated polymer. The fluorinated polymer should have an index of refraction substantially corresponding to the index of refraction of the silica. The difference in index of refraction between the silica stratum and the fluorinated stratum should not exceed about 0.1.

The eighth-wave silica stratum is preferably provided by use of a colloidal silica. Colloidal silica as used herein is intended to refer to aqueous sols of widely dispersed discrete particles which are essentially amorphous silica ( $SiO_2$ ). The silica particles preferably are extremely small, being on the order of about 15 millimicrons or even smaller, e.g., about 7 millimicrons. The silica particles may have a small quantity of sodium ions on the surface to prevent agglomeration. Particularly useful colloidal silicas are the sols of colloidal sil-

ica comprising aqueous colloidal dispersions of surface-hydroxylated silica commercially available from E. I. du Pont de Nemours Co., Wilmington, Del., under the tradename "Ludox" colloidal silica. On dry-down, surface hydroxyl groups on the silica particles induce coalescence and inter-particle bonding results. The index of refraction of such silica strata is about 1.41 to 1.46.

The fluorinated polymer may be selected from among the many well-known and readily synthesizable fluorinated polymers. The index of refraction typically increases as the degree of fluorination is increased. Fluorinated polymers having indices of refraction of about 1.3 to 1.45 are preferred. Good adhesion of the fluorinated polymer to the silica stratum is of course highly desired, and the adhesion ability of any given fluorinated polymer may be readily determined by routine tests, keeping in mind the adhesion desirable for any specific utilization.

In accordance with this invention, the desired quarter-wave anti-reflection layer comprises two eighth-wave layers as illustrated in FIG. 4. The element shown in FIG. 4 has novelty and utility apart from the photographic applications specifically described herein. As shown in FIG. 4, a transparent polyester support 24 has coated on one surface thereof an eighth-wave layer 26a of silica and an eighth-wave layer 26b of a fluorinated polymer. Generally speaking, the two eighth-wave layers 26a and 26b providing the anti-reflection coating 26 will have a combined optical thickness of about 0.08 to about 0.2 micron and more preferably from about 0.12 to about 0.15 micron, or a preferred physical thickness of about 0.09 to about 0.11 micron.

The following example is illustrative of the preparation of an element of the type shown in FIG. 4.

#### Example

A transparent 4 mil polyethylene terephthalate film base 43 inches wide was coated at room temperature with an eighth-wave layer of colloidal silica (dry coverage of silica about 7-8 mg./ft.<sup>2</sup>) by applying a colloidal silica coating solution at an approximate rate of 90 cc./minute with the film base moving at a rate of approximately 50 ft./minute. The colloidal silica coating solution comprised 1.98 liters of an aqueous 1 percent solution of Triton X-100 (tradename of Rohm and Haas Co. for a nonionic wetting agent, isoctyl phenyl polyethoxy ethanol), 1.24 liters of Ludox SM-30 (tradename of E. I. du Pont de Nemours for a colloidal silica dispersion approximately 30 percent by weight silicon dioxide, approximate particle diameter 7 millimicrons) and 23.2 liters of distilled water. The wet silica coating was dried at 250° F. An eighth-wave fluorinated polymer coating was applied at room temperature over the silica layer by applying, at an approximate rate of 130 cc./minute with the film base moving at a rate of approximately 55 ft./minute, a solution comprising 112.9 kg. of methyl ethyl ketone, 28.2 kg. of methyl isobutyl ketone, 2.26 kg. of Kynar 7201 (tradename of Pennwalt Chemical Co. for a copolymer of vinylidene fluoride and tetrafluoroethylene) and 0.399 kg. of polymethyl methacrylate. This coating also was dried at about 250° F., giving a dry coverage of about 9-10 mg./ft.<sup>2</sup>. The polyethylene terephthalate film base contained a small quantity of carbon black to prevent light piping by internal reflection, as described and claimed in the above-mentioned application of Edwin H. Land,

Ser. No. 194,407, filed Nov. 1, 1971. The eighth-wave silica coating was applied to the "raw" film base, i.e., the film base was not given any special treatment prior to coating.

5 While coatings applied were intended to have an eighth-wave thickness with respect to a wavelength of about 5,500 Angstroms, it will be seen from curve B in FIG. 5 that the coatings actually applied resulted in a minimum reflectance at about 6,000 Angstroms. 10 The anti-reflection properties of the just-described anti-reflection coating were determined by applying a flat black coating to the uncoated other surface of the polyethylene terephthalate film base by spraying on a coat of Krylon Ultra Flat Black Enamel No. 1602 Spray 15 Paint. As a control, a similar flat black coating was applied to one surface of another length of the same polyethylene terephthalate film base to which the anti-reflection coating had not been applied. The reflectance of light incident upon the two film bases was 20 measured in a Cary 14 recording spectrophotometer with an integrating sphere. The thus-measured reflectances are reproduced in FIG. 5 wherein curve A is the specular reflectance of the film base without an anti-reflection coating, curve B is the specular reflectance 25 of the film base with the above-described anti-reflection coating, and curve C is the diffuse reflection without the anti-reflection coating. The efficiency of the anti-reflection coating is indicated by the difference between curves A and B, with curve C indicating the 30 minimum reflectance one could hope to obtain. This comparison readily demonstrates the substantial reductions in reflected light provided by the anti-reflection coating applied in accordance with this invention.

The just-described polyethylene terephthalate film base was then used as the support for an image-receiving element of the type shown as element 32 in FIG. 1 and an integral negative-positive multicolor reflection print was prepared in accordance with the procedure described in Example 2 of the copending application of Edwin H. Land, Stanley M. Bloom, and Howard G. Rogers, Ser. No. 246,669, filed Apr. 24, 1972 (now U.S. Pat. No. 3,801,318 issued Apr. 2, 1974). The general format of the integral negative-positive reflection print was similar to that shown in FIG. 1 of the above-mentioned U.S. Pat. No. 3,415,644. Similar films were prepared wherein the polyethylene terephthalate film base carried (a) a quarter-wave layer of colloidal silica (Ludox SM) or (b) a quarter-wave layer of the above described Kynar-polymethyl methacrylate mixture. Good anti-reflection properties were obtained with all three types of anti-reflection coatings. When the respective film units were processed in a Polaroid SX-70 Land Camera, it was found that the film carrying the two eighth-wave coatings exhibited the greatest resistance to scratching during film advance from the cassette through the processing rollers to exit from the camera. It was unexpected that the use of two eighth-wave coatings would give greater resistance to scratching than either of the same materials present as a quarter-wave layer. This result was particularly unexpected in view of the fact that a quarter-wave coating of silica exhibited a tendency to be brittle and flake off, and a quarter-wave coating of the Kynar fluorinated polymer exhibited marginal adhesion in a Scotch tape adhesion test. The film carrying the two eighth-wave coatings exhibited at least as good resistance to scratching during film ad-

vancement as the uncoated polyethylene terephthalate film base.

The unexpectedly greater adhesion and resistance to scratching noted in the above tests using an eighth-wave layer of silica was demonstrated with eighth-wave layers of other fluorinated polymers, e.g., Fluoropolymer B (tradename of E. I. du Pont de Nemours for a 70/20/10 copolymer of vinylidene fluoride, tetrafluoroethylene and vinyl butyrate, Viton A (tradename of E. I. du Pont de Nemours for a 30/70 copolymer of hexafluoropropylene and vinylidene fluoride, and Kel F Elastomer 3,700 (tradename of 3M Company for a 50/50 copolymer of chlorotrifluoroethylene and vinylidene fluoride.

As noted above, the product shown in FIG. 4 has utility apart from use as a photographic film support. One such use is a protective sheet laminated, anti-reflection coating outermost, to the surface of a processed photographic image, e.g., a diffusion transfer image, in accordance with the teachings of U.S. Pat. No. 2,798,021 issued July 2, 1957 to Edwin H. Land. It is also within the scope of this invention to apply the same anti-reflection coating to both surfaces of the transparent support, especially where the product is not intended for use as a photographic film support, e.g., for use as protective transparent covers for notebook pages.

It will be recognized by those of ordinary skill in the art that the solvent of choice for a particular material, and the concentration of the material in the coating solution, may be readily determined by routine experimentation. Obviously the solvent should be one which will not adversely affect, mechanically or optically, the transparent support upon which it is coated.

The transparent support advantageously has a moisture permeability rate adapted to accelerate "drying" of the layers forming the integral negative-positive reflection prints of the preferred embodiments. Reference may be made to U.S. Pat. No. 3,573,044 issued Mar. 30, 1971 to Edwin H. Land for a detailed description of dimensionally stable, transparent supports, e.g., microporous polyesters, having suitable permeability rates, and said description is hereby incorporated herein for convenience. It will be understood that selection of an anti-reflection coating should not adversely affect the desired moisture transmission rate of the transparent support(s).

While the image dye-providing material is generally carried on the same support as the photosensitive silver halide, it will be understood that this initial location is not essential, as in forming monochromes the image dye-providing material may initially be contained in the processing composition or in a layer of the image-receiving element as is taught, for example, in the use of dye developers in the previously mentioned U.S. Pat. No. 2,983,606.

The provision of an anti-reflection coating provides a number of advantages. In the absence of the anti-reflection coating provided in accordance with this invention, the optimum angle for viewing an image through the transparent support is very specific and limited, if the viewer is to avoid to the maximum possible extent seeing specular reflection from the surface of the transparent support of light from the illumination source. The anti-reflection coating has been found to substantially reduce or prevent such specular reflection, thus greatly improving viewing. The resulting images exhibit, as shown above, increased color satura-

tion and density and "cleaner" whites, i.e., reduced minimum densities. The avoidance of light loss during photoexposure is useful also in films wherein exposure is effected through a transparent support but the final image is separated and not viewed through a transparent support. The reduction in surface reflection (glare) simplifies copying integral negative-positive reflection prints of the type with which this invention is primarily concerned and aids in obtaining truer copy prints; light polarizers are customarily used to eliminate surface glare during copying. The anti-reflection coating may also provide anti-abrasion protection and, depending upon the polymer or other material used, desirable anti-friction properties to facilitate transport during manufacture and/or processing.

It is recognized that anti-reflection coatings have been used on photographic prints previously, e.g., U.S. Pat. No. 3,617,354 proposes to apply a layer of a polymerized perfluorinated olefin over the image-bearing photographic emulsion layer of a photographic print. The "photographic emulsion layer" referred to is customarily gelatin, and that patent acknowledges that only limited reduction of surface reflection is possible because such perfluorinated polyolefins do not have indices of refraction low enough to equal the ideal low index of about 1.23 required in view of gelatin's typical index of about 1.5. In contrast, the preferred and most useful embodiments of the present invention apply the anti-reflection coating to a polymeric layer having a much higher index of refraction; the seeming disadvantage of such high indices of refraction as about 1.66 for a polyester transparent layer thus becomes a distinct advantage as the resulting "ideal" index of refraction for an anti-reflection coating becomes more practical to provide. For this reason, an anti-reflection coating of a given "low" index of refraction will provide a greater reduction in glare and surface reflection from a high index polyester than from a lower index polymer such as cellulose acetate. (It will be understood, however, that the present invention expressly includes the use of cellulose acetate as well as polyester and other high index transparent films.)

Furthermore, the teachings of the prior art as illustrated by said U.S. Pat. No. 3,617,354 require that the anti-reflection coating be applied after the final image is formed, to avoid interference with processing solutions or chemicals, e.g., by virtue of impermeability or low permeability to aqueous solutions as would be true of perfluorinated polyolefin coatings. Other efforts to provide anti-reflection coatings by aftertreatment have resulted in coatings which reduce glare but also reduce density by virtue of a coating which is not optically continuous and/or not optically clear.

It also is recognized that the use of silica to provide matte surfaces, thereby reducing glare, previously has been proposed. Such matte anti-reflection layers function by different principles, e.g., light-scattering, and are totally different in visual appearance and effect from the anti-reflection coatings of the present invention. Thus, for example, while a matte surface reduces glare it also reduces the visual color saturation of the image, and its presence is visually apparent. In contrast, the anti-reflection coating of the present invention is almost, if not completely, invisible, and it thus permits the color saturation of the image to be seen without the dilution introduced by either a glossy surface or a matte surface.

Where the expression "positive image" has been used, this expression should not be interpreted in a restrictive sense since it is used primarily for purposes of illustration, in that it defines the image produced on the image-carrying layer as being reversed, in the positive-negative sense, with respect to the image in the photosensitive emulsion layers. As an example of an alternative meaning for "positive image," assume that the photosensitive element is exposed to actinic light through a negative transparency. In this case, the latent image in the photosensitive emulsion layers will be a positive and the dye image produced on the image-carrying layer will be a negative. The expression "positive image" is intended to cover such an image produced on the image-carrying layer.

Since certain changes may be made in the above product and process without departing from the scope of the invention herein involved, it is intended that all matter contained in the above description or shown in the accompanying drawings shall be interpreted as illustrative and not in a limiting sense.

What is claimed is:

1. A photographic product for use in diffusion transfer processes comprising a transparent support carrying on one side thereof an image-receiving layer, the other side of said transparent support carrying an anti-reflection coating having an index of refraction at least about 0.20 less than said transparent support, said anti-reflection coating comprising a stratum of a fluorinated polymer over a stratum of silica, each said stratum having an optical thickness approximately an eighth-wave thick, the indices of refraction of said fluorinated polymer and said silica differing by not more than about 0.1.

2. A photographic product as defined in claim 1, including at least one layer containing photosensitive silver halide carried on said first side.

3. A photographic product as defined in claim 2, including an image dye-providing material in a layer contiguous to said silver halide containing layer.

4. A photographic product as defined in claim 1 wherein said image-receiving layer includes a mordant for a dye.

5. A photographic product as defined in claim 1 wherein said image-receiving layer is a silver receptive layer containing a silver precipitant.

6. A photographic product as defined in claim 4 wherein said dye is a dye developer.

7. A photographic product as defined in claim 1 wherein said transparent support has an index of refraction of at least about 1.6.

8. A photographic product as defined in claim 7 wherein said transparent support is a polyester.

9. A photographic product as defined in claim 8 wherein said polyester is polyethylene terephthalate.

10. A photographic product as defined in claim 7 wherein said anti-reflection coating has an index of refraction of about 1.3 to about 1.45.

11. A photographic product as defined in claim 1 wherein said transparent support is cellulose acetate.

12. A photographic product as defined in claim 7 wherein said silica stratum comprises silica particles having a diameter of about 15 millimicrons.

13. A photographic product as defined in claim 7 wherein said silica stratum comprises silica particles having a diameter of about 7 millimicrons.

14. A photographic product as defined in claim 7 wherein said fluorinated polymer is a vinylidene fluoride copolymer.

15. A photographic product as defined in claim 14 wherein said fluorinated polymer is a copolymer of vinylidene fluoride and chlorotrifluoroethylene.

16. A photographic product as defined in claim 14 wherein said fluorinated polymer is a copolymer of vinylidene fluoride and tetrafluoroethylene.

17. A photographic product as defined in claim 14 wherein said fluorinated polymer is a copolymer of vinylidene fluoride and hexafluoropropylene.

18. A photographic product comprising a transparent support carrying on one side thereof a layer containing

15 a photosensitive silver halide, said silver halide layer being exposable through said transparent support, the other side of said transparent support carrying an anti-reflection coating having an index of refraction at least about 0.20 less than said transparent support, said anti-

20 reflection coating comprising a stratum of a fluorinated polymer over a stratum of silica, each said stratum having an optical thickness approximately an eighth-wave thick, the indices of refraction of said fluorinated polymer and said silica differing by not more than about 0.1.

25 19. A photographic product as defined in claim 18, including an image dye-providing material in a layer contiguous to said silver halide containing layer.

20 30 20. A photographic product as defined in claim 19 wherein said image dye-providing material is a dye developer.

35 21. A photographic product as defined in claim 19 wherein said image-dye providing material is a compound which provides a diffusible dye as a function of oxidation or color coupling.

22. A photographic product as defined in claim 18 including an image-receiving layer, said layer of silver halide being positioned between said support and said image-receiving layer.

40 23. A photographic product as defined in claim 18 wherein said transparent support has an index of refraction of at least about 1.6.

24. A photographic product as defined in claim 23 wherein said transparent support is a polyester.

25 45 25. A photographic product as defined in claim 23 wherein said anti-reflection coating has an index of refraction of about 1.3 to about 1.45.

26. A photographic film product comprising a first support and a second support, at least one of said supports being transparent, a plurality of layers including a photosensitive silver halide layer carried on one of said supports, and a rupturable container releasably holding a processing composition adapted, when distributed between a pair of predetermined layers carried by said supports, to develop said photosensitive layer and provide an image viewable through said transparent support, the external surface of said transparent support carrying an anti-reflection coating having an index of refraction at least about 0.20 less than said transparent support, said anti-reflection coating comprising a stratum of a fluorinated polymer over a stratum of silica, each said stratum having an optical thickness approximately an eighth-wave thick, the indices of refraction of said fluorinated polymer and said silica differing by not more than about 0.1.

60 65 27. A photographic product as defined in claim 26 wherein both of said supports are transparent and each

said transparent support carries said anti-reflection coating on the external surface thereof.

28. A photographic product as defined in claim 26, including an image-receiving layer and means adapted to provide a masking layer between said photosensitive layer and said image-receiving layer to mask the developed photosensitive layer when the image in said image-receiving layer is viewed through said transparent support.

29. A photographic product as defined in claim 28 wherein said product includes a silver halide solvent and said image is a silver transfer image.

30. A photographic product for forming a diffusion transfer image in dye within a permanent laminate including at least one developed silver halide layer, said photographic product comprising, in combination, an image-receiving layer; at least one silver halide emulsion, each said silver halide emulsion having associated therewith an image dye-providing substance selected from the group consisting of image dyes and image dye intermediates; means providing a light-reflecting layer between said image-receiving layer and said silver halide emulsion(s) to mask said silver halide emulsion(s) after development thereof and to provide a white background for viewing a dye image in said image-receiving layer; a transparent support through which image-receiving layer may be viewed; means providing a processing composition for developing said silver halide emulsion(s) after photoexposure and for forming a transfer image in at least one dye in said image-receiving layer; said product including an anti-reflection coating on the outer surface of said transparent support having an index of refraction at least about 0.20 less than said transparent support, said anti-reflection coating comprising a stratum of a fluorinated polymer over a stratum of silica, each said stratum having an optical thickness approximately an eighth-wave thick, the indices of refraction of said fluorinated polymer and said silica differing by not more than about 0.1.

31. A photographic film as defined in claim 30 wherein each said dye is a dye developer.

32. A photographic film as defined in claim 30 wherein each said image dye-providing substance is an intermediate for an image dye.

33. A photographic product as defined in claim 30 wherein said silver halide emulsion(s) are adapted to be exposed through said transparent support.

34. A photographic product as defined in claim 30 wherein said means providing a light-reflecting layer comprise a white pigment dispersed in said processing composition, and said processing composition is contained in a rupturable container positioned to distribute said processing composition containing said pigment between said image-receiving layer and said silver halide emulsion(s).

35. A photographic product as defined in claim 30 comprising a temporary laminate including said layers confined between two dimensionally stable supports, at least one of said supports being transparent, the bond between a predetermined pair of layers being weaker than the bond between other pairs of layers, and including a rupturable container releasably holding said processing composition, said rupturable container being so positioned as to distribute said processing composition between said predetermined layers, said processing composition being adapted to provide said

permanent laminate following distribution and drying.

36. A photographic product as defined in claim 30 wherein said transparent support has an index of refraction of at least about 1.6.

37. A photographic product as defined in claim 36 wherein said transparent support is a polyester.

38. A photographic product as defined in claim 37 wherein said polyester is polyethylene terephthalate.

39. A photographic product as defined in claim 36 wherein said anti-reflection coating has an index of refraction of about 1.3 to about 1.45.

40. A photographic product comprising a first support; a red-sensitive silver halide emulsion; a green-sensitive silver halide emulsion; and a blue-sensitive silver halide emulsion; said silver halide emulsions having associated therewith, respectively, a cyan dye developer, a magenta dye developer and a yellow dye developer; an image-receiving layer for receiving image dyes transferred thereto by diffusion as a function of exposure and development of said silver halide emulsion layers; a second support which is transparent and through which said image-receiving layer may be viewed; a rupturable container releasably holding a processing composition adapted, upon distribution between predetermined layers of said film to develop said silver halide emulsions and to effect the formation of a transfer image in dye in said image-receiving layer, said processing composition also being adapted to provide

20 a permanent laminate including said developed silver halide emulsions and said image-receiving layer; and means providing a light-reflecting layer between said image-receiving layer and said silver halide emulsions effective to provide a white background for viewing said transfer image and for masking said developed silver halide emulsions; said product including an anti-reflection coating on the outer surface of said transparent support having an index of refraction at least about 0.20 less than said transparent support, said anti-reflection coating comprising a stratum of a fluorinated polymer over a stratum of silica, each said stratum having an optical thickness approximately an eighth-wave thick, the indices of refraction of said fluorinated polymer and said silica differing by not more than about 0.1.

30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 987

container being so positioned as to release said processing composition for distribution between said pair of layers.

47. A photographic product as defined in claim 40, wherein said silver halide emulsions are present as separate planar layers.

48. A photographic product as defined in claim 40, wherein said silver halide emulsions are present in the form of minute elements arranged in side-by-side relationship in a photosensitive screen pattern.

49. A photographic product as defined in claim 47, wherein said blue-sensitive silver halide emulsion layer is between said image-receiving layer and said other silver halide emulsion layers.

50. A photographic product as defined in claim 47, wherein said blue-sensitive silver halide emulsion layer is between said first support and said other silver halide emulsion layers, and said first support is transparent.

51. A photographic product as defined in claim 50 wherein said transparent first support carries an anti-reflection coating on the outer surface thereof having an index of refraction at least about 0.20 less than said transparent support, said anti-reflection coating comprising a stratum of a fluorinated polymer over a stratum of silica, each said stratum having an optical thickness approximately an eighth-wave thick, the indices of refraction of said fluorinated polymer and said silica differing by not more than about 0.1.

52. A photographic laminate comprising (a) at least one exposed and developed silver halide layer, (b) an image-carrying layer containing an image in at least one dye, (c) a light-reflecting, white layer positioned between said silver halide layer or layers and said image-receiving layer and effective to mask said developed silver halide layer or layers, and (d) a transparent layer through which said image may be viewed against said white layer, said layers being permanently laminated together, said transparent layer having an anti-reflection coating on the outer surface thereof, said anti-reflection coating having an index of refraction at least about 0.20 less than said transparent layer, said anti-reflection coating comprising a stratum of fluorinated polymer over a stratum of colloidal silica, each said stratum having an optical thickness approximately an eighth-wave thick, the indices of refraction of said fluorinated polymer and of said silica differ by not more than about 0.1.

53. A photographic laminate as defined in claim 52 wherein said transparent layer is a polyester.

54. A method of forming a diffusion transfer dye image by developing an exposed silver halide emulsion, forming an imagewise distribution of a diffusible dye image-providing substance as a function of said devel-

opment, and transferring at least a portion of said imagewise distribution of diffusible dye image-providing substance to an image-receiving layer in superposed relationship with said silver halide emulsion to provide said dye image, said image-receiving layer and said silver halide emulsion forming a permanent laminate including a light-reflecting layer positioned between said image-receiving layer and said silver halide emulsion, the step of said exposure of said silver halide emulsion being effected through a transparent support having an anti-reflection coating on the outer surface thereof, said anti-reflection coating having an index of refraction at least about 0.20 less than said transparent support and comprising a stratum of a fluorinated polymer over a stratum of silica, each said stratum having an optical thickness approximately an eighth-wave thick, the indices of refraction of said fluorinated polymer and said silica differing by not more than about 0.1.

55. A method as defined in claim 54 wherein said diffusion transfer dye image is viewed through said transparent support and said anti-reflection coating.

56. A method as defined in claim 54 wherein said diffusible dye image-providing substance is a dye developer.

57. The method as defined in claim 54 wherein a red-sensitive silver halide emulsion, a green-sensitive silver halide emulsion and a blue-sensitive silver halide emulsion are present, said silver halide emulsions having associated therewith, respectively, a cyan dye developer, a magenta dye developer, and a yellow dye developer, and said dye image is a multicolor image.

58. A photographic image comprising a transparent support carrying on one side thereof an image-carrying layer containing an image in dye or silver, the other side of said transparent support carrying an anti-reflection coating having an index of refraction at least about 0.20 less than said transparent support, said dye image being viewable through said anti-reflection coating and said transparent support, said anti-reflection coating comprising a stratum of a fluorinated polymer over a stratum of silica, each said stratum having an optical thickness approximately an eighth-wave thick, the indices of refraction of said fluorinated polymer and said silica differing by not more than about 0.1.

59. A photographic image as defined in claim 58 wherein said transparent support has an index of refraction of at least 1.6 and said anti-reflection coating has an index of refraction at least about 0.20 less than said transparent support.

60. A photographic product as defined in claim 58 wherein said anti-reflection coating has an index of refraction of about 1.3 to about 1.45.

\* \* \* \* \*